

July 16, 1940.

G. ELLIS

2,208,511

METHOD OF MAKING DENSE WALL PANELS

Filed March 11, 1938



INVENTOR.  
GEORGE H. ELLIS  
BY  
H.F. Woodward  
ATTORNEY.

## UNITED STATES PATENT OFFICE

2,208,511

## METHOD OF MAKING DENSE WALL PANELS

George H. Ellis, New Brighton, Minn., assignor to  
The Insulite Company, Minneapolis, Minn., a  
corporation of Minnesota

Application March 11, 1938, Serial No. 195,353

7 Claims. (Cl. 92—39)

This invention relates generally to a process of making hard, dense board, slabs or panels and particularly to such bodies which have high strength both wet and dry and have a small coefficient of expansion in the presence of moisture.

An object of the invention is to produce in a shorter time composite bodies or sheets adapted for use in construction of building and for various other uses.

Another object of the invention is to provide an improved process for making board or sheets in which high temperatures are used and the body is moved along continuously.

Another object is the production of bodies of various types from fibrous vegetable material of any desired length, width and thickness.

The invention relates to the production of hard, stiff bodies by first forming from vegetable fibrous pulp stock a body, removing the surplus moisture from the body, passing the body through a heater to remove the moisture, heating the body to raise the temperature thereof with comparatively light pressure, applying higher temperatures, a relatively high pressure for a relatively short time and then quickly chilling the hot pressed body. The last step may be omitted but it is preferred that it be used.

In carrying out the process water-proofing material and/or binders may be added but they may be omitted if desired and a good product obtained.

With the foregoing and other objects in view the invention consists of the novel steps and combination of steps hereinafter more specifically described and illustrated in the accompanying drawing wherein is shown embodiments of the invention but it is to be understood that changes, variations and modifications may be resorted to which fall within the scope of claims hereunto appended.

In the accompanying drawing:

Figure 1 is a vertical section through an apparatus showing a view diagrammatically illustrating such apparatus for making composition boards, sheets or bodies which includes a felting device, a wet press, a high temperature dryer, a heat and hot pressing device.

In Figure 1A is a vertical section view of the pressing rolls and chilling rolls.

Referring to the drawing in detail, 10 indicates a head box for receiving the vegetable fibrous pulp, 11. Operatively mounted adjacent the head box are forming rolls 13 and 14 which pick up the fibers and form them into a continuous sheet.

Flexible members 12 and 15 are secured to the

head box 10 and are adapted to contact the forming rolls 13 and 14 respectively.

Sheet 16, formed by rolls 13 and 14, is passed to a suitable wet press to remove the surplus moisture. The wet press consists of belts 17 and 18, mounted upon rolls 19, 20, 21, 22, 24 and 25. Rolls 23 are for the purpose of maintaining proper tension on the belts 17 and 18.

The sheet 16, after having the surplus moisture removed by the wet press, is passed to a suitably constructed dryer. The dryer may be single tier or, if desired, may be multiple tier. The drier consists of upper section 26 and lower section 27. In the upper part of the dryer is located heating coils 28 while the heating is supplied to the lower section by heating coils 29. The temperature of the dryer is preferably around 600° F. to 700° F. on the wet or receiving end and 300° F. to 450° F. on the discharge or dry end.

The sheet 16 may be divided at "B" after being discharged from the dryer. The moisture contents of the sheet as it comes from the dryer may be bone dry but for an economical operation it is preferred that the moisture contents be within the range of 2 to 10%.

The dry sheet, whether bone-dry or air-dry is passed to a preheating press consisting of sections 31 and 32 in which are mounted heating rolls 33 and 34. The temperature maintained in the preheater presser should be within the range of 400° F. to 500° F., preferably about 425° F. Preferably only surface contact pressure is applied in the preheater presser. The board or product in the preheater has the constituents of the vegetable material rendered substantially plastic.

One or more pairs of large hot pressing rolls, 39 and 40, are positioned adjacent the discharge end of the preheating press. The rolls 39 and 40 are heated by any suitable means as for instance by steam introduced through members 43 and 44. The waste steam is withdrawn from rolls 39 and 40 through the medium of conduits 37 and 38. The conduits 37 and 38 discharge the waste heat through headers 35 and 36, into the preheater press.

The large pressing rolls 39 and 40 are heated from 500° F. to 575° F., preferably about 550° F. The vegetable material contained in the board at the time it reaches the large rotatable pressing members is in a highly plastic condition. The pressure applied by rolls 39 and 40 varies in accordance with the kind of product desired from 500# per square inch to 2000# per square inch. Generally to obtain a product that has a tensile

strength above 6000 pounds per square inch, a pressure of about 1000# per square inch is employed.

The pressed and hot board, 45, may be divided into suitable lengths by means of cut-off member 46. In the preferred process the board as discharged from the large hot pressing rolls is passed between cooling or chilling rolls. The chilling rolls may be maintained in a cold condition by any suitable means. The hot pressed board which has the temperature quickly brought down below the plastic point of the substance contained in the vegetable material is of greater density, has higher wet and dry strength and absorbs less water than a board not thus cooled.

Any suitable vegetable material can be used and the method of reducing the vegetable material to a pulpy condition can be by grinding, crushing or any desired method. The pulp used in producing the new products of this invention should be raw or semi-chemical, that is, should be produced by mechanical means or by a relatively light cooking process.

If desired, material from an extraneous source such as vegetable oil or material, mineral oils or material, and animal oils may be incorporated in the product to increase the water resistance. Hydrogenated whale oil in an amount from 1% to 5% has given excellent results and decreases the water absorption about 50% over a product not having the oil incorporated therein. If a material from an extraneous source is incorporated in the product it is preferred that such material have the character of hardening under heat and pressure.

Should whale oil be used it is generally commingled with the vegetable fibers while in a water suspension. The drying of the board to remove substantially all the moisture without pressure 40 preliminarily heat treats the oil which permits of a rapid hardening under heat and pressure.

If board-like bodies are to be produced by this process, the time for completing the board is about one-half the time required by known processes. The strength and other qualities of the products produced in accordance with the process hereinbefore described are very much higher than any heretofore made.

The surface of the products produced by my process is smooth, highly polished and does not have surface pores that can be detected by the eye. The heat-hardening products of the vegetable material being pressed flow to the surface of the product and give it a high surface strength and water resistance. The surface on the products made by my process has great resistance to surface abrasion, in fact, substantially four times the resistance of any known pressed board.

The following is one example for producing board-like bodies: Wood is reduced to pulp by the grindstone method. Three per cent of whale oil is commingled with the pulp while in a water bath by passing the oil and pulp through a Jordan. A thick sheet is formed and the surplus moisture is removed and the sheet is passed to a high temperature dryer where substantially all the moisture is removed or at least has the moisture removed down to an air dry condition. The dry board is then passed through the preheater 60 press, the temperature in the preheater being about 440° F. The board becomes heated throughout and becomes quite plastic. The rollers or rotatable members compress the board very little as only surface contact is maintained. The hot board is quickly compressed to its sub-

stantial final thickness by the large heated rotatable members. The pressed board is then quickly chilled by cooling rolls. The sheet, board or product is in continuous motion from the time the product is formed until completed.

If vegetable oils or mineral water-proofing materials are incorporated with the pulp, they receive a preliminary heat treatment when the board or product is dried, which permits of quick hardening under heat and pressure. It is unnecessary when using my process to heat cure the finished product.

It is to be understood that variation and modification can be resorted to which fall within the scope of the appended claims.

It is preferred that a portion of the high temperature dryer be provided with top rolls or rotatable members 30'. The moisture of the board at the time the top rolls are applied usually is and should be about 30% or lower. The rolls 30', smooth or iron the surfaces of the board and also result in utilizing that portion of the vegetable material which can be termed water-soluble, hardening material. Such materials harden as the moisture leaves it as is the case of ordinary 23 glue.

The board discharged from the dryer has a substantially smooth surface or surfaces and the water-soluble binder is set. The board discharged from the dryer can be used if high strength 30 smooth surface insulating products are desired. The board or product thus produced has relatively high insulating value and at the same time has higher wet and higher dry strength than any known insulating board.

To obtain a very dense and rigid board, the board or product discharged from the dryer is then passed to the preheater press and subjected to the additional steps as shown by the drawing and hereinbefore described.

The boards discharged from the large heating rolls, 39 and 40, are not permitted to materially cool until they reach the chilling rolls. The chilling of the boards under pressure, results in setting up those parts of the vegetable material 45 that harden upon cooling. Thus by this method, all the natural cementing materials of the vegetable materials that act as a binder are utilized.

It is possible to use physical condensation products from an extraneous source as well as chemical condensation products due to the fact of chilling the hot pressed board. What is intended to be covered by the term physical condensation products are binders and/or waterproofing materials that harden by cooling. By chemical condensation products, it is intended to cover heat hardening binders and/or waterproofing materials.

The waste heat from the preheater press may be withdrawn as at C, and discharged into the dryer 60 and the waste heat from the dryer may be withdrawn as at D and used for heating the water suspension of the vegetable fibers prior to forming of the sheet or board.

Board produced in accordance with this process 65 has higher surface resistance to abrasion, higher wet strength after soaking in water for forty-eight hours, and higher dry strength than any known pressed fiber product.

Any vegetable fibrous material may be used in 70 the process and it is intended to include woods of various kinds and fibers obtained from annual plants. Whatever kind of wood or woody material is used, it is preferred that the major portions of the natural cementing materials be in 75

the fiberized material when pressure is applied.

What I claim is:

1. A process of making board-like bodies from raw vegetable fibers which includes commingling approximately 3% of whale oil with fiber in a water suspension, forming a board from the fibers, pressing the sheet to remove the surplus moisture, drying the sheet without pressure to reduce the moisture content to about 30%, thereafter ironing the surface of the board while continuing the drying, then applying surface contact pressure at a temperature of about 400° to 460° F. to the board having a moisture content from 2 to 10%, thereafter applying pressure of at about 500 pounds per square inch to the dry board at a temperature of about 500° to 575° F., and finally quickly chilling the board to lower the temperature whereby the board is cemented together by natural cementing material contained in the fibers.
2. A process of making board-like products from vegetable fiber containing substantially all of the natural cementing materials of the original vegetable material comprising drying a wet board-like product without application of pressure, applying surface contact pressure only by rotatable means at a temperature of about 400° F. to 500° F., then applying pressure of at least 500 pounds per square inch at a temperature of about 500° to 575° F., and thereafter quickly chilling the hot board-like product under pressure by means of rotatable members.
3. A continuous process of making board-like bodies which comprises forming a board from vegetable fibers in a water suspension, pressing the board to remove the surplus moisture, advancing the board through a dryer, smoothing the surface of the board in the dryer after the moisture content has been reduced to below 30%, then heating the substantially dry board while maintaining surface contact with the moving board by rotatable members at a temperature above 400° F., applying high pressure to the hot and dry board at a temperature of about 500° to 575° F., and then quickly reducing the temperature of the hot pressed board by passing the board between chilling members.
4. A process of making hard, highly water-resisting, and dense board-like bodies which includes commingling hydrogenated whale oil with fibers in a water suspension, passing a mixture of pulp and oil through a Jordan to substantially

uniformly coat the fibers with oil, forming a board, pressing the board to remove the surplus moisture, drying the board without pressure to reduce the moisture contents, ironing the surfaces of the board after the moisture contents have been reduced to about 30% while continuing the drying, then heating the board at a temperature of about 400° F. to 500° F. with light surface contact pressure, and pressing the hot board at a temperature within the range of 500° to 575° F. at a pressure from 500 to 2000# per square inch.

5. A process of making hard, dense and highly water-resistant board-like bodies from vegetable fibers in a water suspension, commingling a water-proofing material with the fibers, forming a board-like body, removing the surplus moisture, drying the board without pressure, then smoothing the surface of the board during drying after the moisture has been reduced to about 30%, then applying only surface contact pressure at a temperature within the range of about 400° F. to about 500° F., thereafter applying consolidating pressure at a temperature above 500° F. and then quickly chilling the hot board under pressure.

6. A process of making board-like products including the steps of forming a felted board from vegetable fibrous material in a water suspension, removing the surplus moisture, drying the board to reduce contents to substantially air dry condition, then heating the board at a temperature of about 400° F. to 500° F. with only surface contact pressure to render the vegetable material hot and plastic, thereafter applying consolidating pressure at a temperature above 500° F., and then quickly chilling the hot board under pressure.

7. The process of making hard and highly water-resistant board having high tensile strength, including the steps of mixing a water-proofing material with vegetable fibers in a water bath, pressing a board to reduce the moisture contents, drying the board and smoothing the surface of the board during drying after the moisture contents have been reduced to about 30% but above 15%, then applying light pressure to the substantially dry board at a temperature of about 400° to 500° F., applying 500 to 2000# per square inch at a temperature above 500° F. to the hot, dry board, and cold pressing the hot board to quickly reduce the temperature below 212° F.

GEORGE H. ELLIS.